

J. F. MONNOT,  
PROCESS OF AND APPARATUS FOR MAKING COMPOUND METAL OBJECTS.  
APPLICATION FILED APR. 17, 1907.

905,558.

Patented Dec. 1, 1908.



**WITNESSES:**

86 Bruce.

A. M. Haughton

**INVENTOR**

INVENTOR  
*J. F. Marrot*

BY

Marble & Eddy  
ATTORNEYS

## ATTORNEYS

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## PROCESS OF AND APPARATUS FOR MAKING COMPOUND METAL OBJECTS.

No. 905,558.

Specification of Letters Patent.

Patented Dec. 1, 1908.

Application filed April 17, 1907. Serial No. 368,654.

To all whom it may concern:

Be it known that I, JOHN F. MONNOT, a citizen of the United States, residing at New York, in the county of New York and State 5 of New York, have invented certain new and useful Processes of and Apparatus for Making Compound Metal Objects; and I do hereby declare the following to be a full, clear, and exact description of the same, such as will 10 enable others skilled in the art to which it appertains to make and use the same.

My invention relates to processes of and apparatus for producing compound metal objects, comprising unlike metals, such for 15 example as iron and copper, iron and silver, iron and brass, etc., united by a union which is, or which is substantially equivalent to, a true weld.

In applications Sr. Nos. 281,680 and 20 333,570, heretofore filed by me, I have set forth a discovery made by me which is that copper, silver and certain other metals of high melting point which do not unite inseparably to iron and other steel and the like, 25 under ordinary conditions, even when cast at ordinary casting temperatures into contact with such iron or steel, become capable of uniting with iron and steel if heated to a temperature much above the melting point 30 and probably, in the case of copper and silver, from 2500° to 2800° Fahrenheit or higher; the metal when heated to such high temperature appearing to become reactive so as to be capable of entering into direct 35 permanent union with the iron or steel, the union produced being, or being equivalent to, a true weld; and being so firm that the joined metals of the resulting article may not be separated by temperature changes 40 short of an actual melting of one of them, nor can the one metal be stripped from the other by a cutting tool such as a cold chisel; the cutting tool if applied at the line of juncture, failing to follow such line, as would be 45 the case if the metals were not truly united. To the condition of these metals at which they become capable of entering into permanent unions as described, I have applied the term "supermolten condition". In my 50 said application Sr. No. 333,570 I have illustrated and described, and in other applications have claimed, apparatus for producing compound metal objects by dipping an object of one metal into molten bodies of other.

metal or metals and confining a layer of such 55 molten metal of suitable thickness in contact with the said object and permitting such layer to solidify thereagainst; the confining of such metal being commonly performed by what I have termed "segregation". In practice the segregation method 60 of forming coatings from molten metal is most easily carried out with a segregating casing mounted vertically; which in turn requires very deep crucibles, when ingots of 65 considerable size are to be coated; and these crucibles are somewhat expensive, and likewise the deep body of molten metal within them subjects the crucibles, necessarily weakened by the high temperature to which 70 they are exposed, to excessive pressure.

By the method and apparatus herein described, I am able to produce compound metal bodies such as above referred to, of 75 much larger size than is practicable at present when the vertical form of apparatus shown in my said application Sr. No. 333,570 is used; and I am able to use horizontal and relatively shallow crucibles and to work with the object to be coated in a horizontal position. The method herein described may properly be termed a "displacement" 80 method and will be so referred to herein-after. According to said method, the object to be coated (preferably preheated and 85 protected against oxidation as hereinafter described and, if the operation is carried on in two steps, film coated in the manner hereinafter described,) is lowered in a horizontal 90 position into a relatively shallow crucible or bath of molten metal. Displacement bodies are then lowered into such crucible alongside of such object but spaced therefrom by a distance corresponding to the thickness of coating desired, such displacement bodies 95 being so shaped as to fill the crucible except for the space corresponding to the desired coating. As these displacement bodies are forced down into the crucible they force out through suitable openings, the molten metal 100 in the crucible except the portion thereof in the space between the object to be coated and said displacement cores. The molten metal is then allowed to solidify, after which the coated ingot is withdrawn and worked 105 by rolling, pressing, hammering or the like, with or without submission to a soaking heating as circumstances require.

In the accompanying drawings I illustrate apparatus which may be used for carrying out the method herein described.

In said drawings: Figure 1 shows a diagrammatic longitudinal section of apparatus for carrying out my invention. Fig. 2 shows a vertical section through the coating crucible and protecting casing. Fig. 3 shows a transverse section through the coating crucible before the displacement bodies are introduced therein, and Fig. 4 is a similar view showing said displacement bodies in place. Figs. 5 and 6 are respectively a detail top view and a detail vertical section 15 of a coating crucible provided with lugs for centering the billet and spacing it up from the bottom of the crucible.

The apparatus shown in these drawings comprises a preliminary heating chamber 1, preferably as shown a closed chamber around which gases may be circulated so as to heat the billets within said chamber without exposing them to oxidizing or deteriorating influences. Such chamber has in its top openings 2 for the removal of the heated billets.

3 is a casing of approximately the shape and size of the said billets but open at the bottom, said casing supported by suitable hoisting means 4 by which it may be raised and lowered. Porter bars 5 pass through openings in the top of this casing and are adapted at their lower ends to engage said billet. They are supported by hoisting means 6; the construction being such that the casing with the billet within it may be raised and lowered as a whole, or the billet may be raised into or lowered from said casing. Said casing is provided with a pipe 7 for the supply of a suitable non-oxidizing, indifferent or protective atmosphere, such as producer gas made from coke, anthracite or charcoal and containing no considerable amount of marsh gas or decomposable hydrocarbons. A valve 8 controls the flow of gas through pipe 7. The hoisting apparatus 4 and 6 are preferably mounted upon a truck 9 running on rails 10 or any other suitable conveying apparatus by which it may be moved from place to place.

11 and 12 are crucibles containing molten metal. 13, 13 are displacement bodies formed of or coated with, suitable refractory material (usually graphite or crucible mixture) and arranged to be raised from and lowered into one of said crucibles by any suitable means, as for example, hoisting means 14 on truck 9 from which is suspended a cross frame 15 to which said displacement bodies are connected.

As will be seen, the crucible 12 corresponds in shape generally to the shape of the billet 16, but is somewhat wider than said billet and has sloping sides 17 and an overflow spout 18. The displacement bodies 13, 13 have simi-

larly inclined sides on the faces away from the billet and toward the sides of the crucible. Said displacement bodies are further provided with spacing lugs 19 near their ends, which lugs are commonly formed of graphite or crucible mixture and are set into recesses in the displacement bodies; and I may provide adjusting means for such lugs, for example, screws 20 inserted from the outer sides of the bodies and with their heads covered over by plugs 21 which may be removed when it is desired to adjust the lugs 19.

I will first describe the method of carrying out the operation by double dipping. In such case, the metal within the crucible 11 may be supermolten metal, and that in crucible 12 may be molten but not supermolten, and at or near ordinary casting temperature; all that is required being that the metal in crucible 12 be quite fluid. It is not necessary that the two crucibles shall contain the same metal and therefore it may happen that although the metal in crucible 11 is supermolten and that in crucible 12 is more near the ordinary casting temperature, yet the metal in crucible 12 may be as hot or even hotter than the metal in crucible 11. The billet 16 having been pre-heated to the proper degree in furnace 1 (it is usually heated to a temperature between a low red and a bright yellow) the cover of chamber 1 is removed, the casing 3 is moved over the opening 2 of said chamber and is filled with its protective atmosphere if not already so filled, the porter bars are lowered through the casing and are engaged with a billet, and then said billet is raised up into the casing; said casing and billet being then moved over the supermolten bath 11, casing and billet being lowered until the casing is just above the surface of the supermolten metal and then the billet being lowered from the casing into the molten metal and after a sufficient time has elapsed for the formation of a film coating on the billet (a few seconds contact usually suffices) said billet is raised again into the casing filled with its protective atmosphere and said casing and billet are then moved over the molten bath 12, the film coated billet is lowered to the molten metal in said bath, the casing is moved out of the way, and then the displacement bodies 13, 13 are lowered into the crucible 12, displacing as they do the excess of molten metal over that required for the coating and confining between themselves and the billet the layers of molten metal required to form the coating.

In Fig. 1 I have shown the apparatus adapted to form coatings on two sides only of the billet; the billet resting at the bottom on the bottom of the crucible and the overflow spout 18 being substantially flush with the top of the billet, the molten metal flowing

over the top of the billet as it passes to said overflow spout.

In Figs. 4-6 I have shown the apparatus adapted for forming coatings on all four sides of the billet, said billet being spaced up a short distance from the bottom of the ingot by spacing pieces 22 near its ends and the overflow trough 18 being a corresponding distance above the upper surface of the billet.

The excess metal having been forced out of the crucible 12, the metal remaining therein is permitted to solidify against the film coated surface of the billet and when set said billet is raised from the crucible, the porter bars disconnected, if not previously disconnected, and the billet is worked, either before or after submission to a soaking heat.

Instead of carrying on the operation by the double dipping method just described, the entire operation may be carried on with but one dipping. In such case the crucible 11 is not required and the metal in crucible 12 is maintained in the supermolten condition. In such case the billet is raised from the pre-heating chamber 1 into the casing 3 as above described, and said casing and billet are moved over the bath 12 and lowered down to the surface of the metal in such bath and then the billet is lowered further into crucible 12 and immediately thereafter the displacement bodies 13, 13 are inserted as above described. The molten metal is allowed to solidify in the crucible (heating being discontinued temporarily) and as soon as set the billet is withdrawn and treated as above described.

I have found that prolonged contact of the billet with metal in the supermolten condition is detrimental to both metals; but opportunity for deterioration of either metal is not afforded even when the operation is carried on by the dipping method just described, because although the molten metal is supermolten when the billet is first introduced, and remains in that condition long enough to unite with the surface of the billet, the chilling action of the billet upon the supermolten metal almost immediately reduces the relatively small mass of molten metal remaining in the crucible after the introduction of the displacement bodies, below the supermolten state; contact of the two metals having then no appreciable injurious effect upon either. I may further hasten the lowering of the molten metal below the supermolten state by circulating water through the displacement bodies 13, to which end these displacement bodies may either be solid blocks of graphite or crucible mixture, with pipes for circulating cooling water embedded therein, or, as indicated in Fig. 4, they may comprise heavy metal cores 24 coated with crucible mixture or graphite, and the rod supporting these

displacement bodies may be hollow and have flexible pipes 26 connected thereto as shown particularly in Fig. 2. There appears to be, between the ordinary molten condition and supermolten condition, a critical point, above which the molten copper, for example, is reactive upon cast iron, and below which it is not particularly reactive. Therefore, if after initial contact of the billet 16 with the supermolten metal, and after the insertion of the displacement bodies, (which when inserted force out of the crucible the greater part of the molten metal therein,) the metal remaining be lowered quickly below this critical point, there can be no injurious action of the copper on the iron or vice versa. It will be observed that in such case the molten metal is being cooled on both sides; on the one side by absorption of heat by the billet 16, and on the other side by absorption of heat by cooling water passed through the displacement bodies or by radiation from the surface of the molten metal and through the walls of the crucible. It will be understood that there is a time contact or conduction factor which determines the permissible duration of contact of the billet with supermolten metal. While the billet is considerably below the temperature of the supermolten metal and is being heated rapidly thereby, the supermolten metal cannot injuriously affect it or be affected in turn injuriously.

In using displacement bodies having means for circulating cooling water through them, I do not circulate such cooling water while the displacement bodies are being introduced, in order that there may be no thickening of the molten metal adjacent the surfaces of these displacement bodies or possible adhesion of molten metal to them; in fact the water pipes or chambers within said displacement bodies are empty when said bodies are first introduced; but when said bodies have reached their proper positions (by which time the contact of the supermolten metal and the billet will ordinarily have continued long enough for the purpose of the process) the cooling water is circulated.

The displacement bodies may have weights 25 to insure or facilitate their descent.

For guiding the casing 3 in its ascent and descent I have provided guides 23.

Since the displacement bodies 13 are wedges having tapering sides on the outside, they may be planed off or resurfaced from time to time, reduction of dimensions thereby occasioned being compensated for by the slightly lower position which such displacement bodies will then assume, due to such reduced dimensions. Instead of resurfacing in this manner the bodies may be resurfaced by applying this coating of crucible mixture from time to time.

The method of and apparatus for uniting metals, above described, is not confined to

production of weld unions or equivalent unions by means of supermolten metal. If mere physical contact of the two metals, such as an ordinary cast union, is desired, the 5 molten metal may be in ordinary casting condition and such molten metal may even be a metal of relatively low casting temperature, such as lead or tin.

What I claim is:—

10 1. The process of coating metal objects which comprises contacting such an object with a body of molten metal and then displacing from proximity to such object substantially all such molten metal except a layer thereof in immediate proximity to the 15 surface of such an object.

20 2. The process of coating metal objects which comprises contacting such an object with a body of molten metal and then displacing from proximity to such object substantially all such molten metal except a layer thereof in immediate proximity to the 25 surface of such object, and causing such layer to solidify on such surface.

25 3. The process of coating metal objects which comprises film-coating such an object, contacting the film-coated surface with a body of molten metal and then displacing from proximity to such object substantially 30 all such molten metal except a layer thereof in immediate proximity to the surface of such object.

35 4. The process of coating metal objects which comprises placing such an object in a bath of molten coating metal and thereafter placing in such bath in proximity to, but at a predetermined distance from, such object, a displacing body of volume adapted to displace the molten metal not between said object and said body.

40 5. The process of coating metal objects which comprises placing such an object in a bath of molten metal contained in a suitable receptacle of volume sufficient to contain an excess of the molten metal, and thereafter lowering into the receptacle, at a predetermined distance from the surface of such object, a displacing body, and thereby displacing from such receptacle any excess of metal 45 therein.

50 6. The process of coating metal objects which comprises placing such an object in a bath of molten coating metal contained in a receptacle having an outwardly sloping side and of sufficient volume to contain an excess of molten metal, and thereafter lowering into the receptacle a displacing body having an oppositely sloping side in contiguity with the said sloping side of said receptacle until said 55 sloping sides are in contact and the predetermined thickness of molten metal is left between said object and displacing body.

60 7. The process of coating metal objects which comprises film coating such an object 65 by contacting it with molten coating metal,

transferring the object to a second bath of molten coating metal and thereafter placing in such bath in proximity to, but at a predetermined distance from, such object a displacing body of sufficient volume to displace the metal not between said object and said body.

70 8. The process of coating metal objects which comprises film coating such an object by means of supermolten metal and surrounding it with molten metal and then displacing from proximity to such body substantially all such molten metal except a layer thereof in immediate proximity to the 75 surface of such body.

80 9. The process of coating metal objects which comprises contacting such an object with supermolten metal of high melting point, withdrawing said object from such contact under conditions precluding oxidation of the film-coating thereby formed, contacting such film-coating with a body of molten metal and then displacing from proximity to such object substantially all such 85 molten metal except a layer thereof in immediate proximity to the surface of such object.

90 10. The process of coating metal objects which comprises contacting such an object with supermolten metal, withdrawing said object from such contact into a chamber containing a protective atmosphere, transferring said object to a body of molten metal and then displacing from proximity to such object substantially all such molten metal except a layer thereof in immediate proximity to the surface of such object.

95 11. The process of coating metal objects which comprises preliminary heating such an object, transferring it under conditions precluding oxidation to a body of molten metal and then displacing from proximity to such object substantially all such molten metal except a layer thereof in immediate proximity to the surface of such object.

100 12. The process of coating metal objects which comprises preliminarily heating such an object, transferring it under conditions precluding oxidation to a body of supermolten metal and then transferring said object, under conditions precluding oxidation, 105 to a body of molten metal and displacing from proximity to such object substantially all such molten metal except a layer thereof in immediate proximity to the surface of such object.

110 13. Apparatus for coating metal objects comprising a receptacle adapted to contain the object to be coated and molten metal surrounding the same, and displacing means adapted for insertion between such object, 115 when in place in said receptacle, and a side of said receptacle, and of size adapting it to displace the molten metal within said receptacle except a layer thereof of predetermined thickness in proximity to said object.

14. Apparatus for coating metal objects comprising a receptacle adapted to contain the object to be coated and molten metal surrounding the same, and having a sloping side surface, and a displacing body having a similarly sloping side and adapted for insertion between said object and the sloping side surface, and of size adapting it to displace the molten metal within said receptacle except a layer thereof of predetermined thickness in proximity to said object.

15. Apparatus for coating metal objects comprising a receptacle adapted to contain the object to be coated and having means for spacing said object from its bottom, and an overflow above the top of such object when in place within it, and a displacing body adapted for insertion between said object and a side of said receptacle and adapted to displace the molten metal between said object and said side except a layer thereof in proximity to the surface of said object.

16. Apparatus for coating metal objects comprising a displacing body having spacing lugs for spacing it away from the object to be coated.

17. Apparatus for coating metal objects

comprising a displacing body having adjustable spacing lugs for spacing it away from the object to be coated.

18. Apparatus for coating metal objects comprising a displacing body having spacing lugs fitting within recesses of such body and screws for adjusting the same and means for covering the ends of said screws.

19. Apparatus for coating metal objects comprising a displacing body having a sloping surface on one side and having means for spacing it a predetermined distance from the object to be coated.

20. Apparatus for coating metal objects comprising a receptacle for molten metal, a protective casing, means for raising and lowering the same, a displacing body, means for raising and lowering the same out of and into said receptacle, and means for raising into and lowering from said casing an object to be coated out of and into said receptacle.

In testimony whereof, I affix my signature in the presence of two witnesses.

JOHN F. MONNOT.

Witnesses:

BYRON E. ELDRED,  
K. P. McELROY.